

June 22, 1926.

1,589,589

Y. A. DYER

PROCESS AND APPARATUS FOR MELTING IRON

Filed Feb. 4, 1925



Inventor

Yulee A. Dyer  
By Charles O. Hanes  
his Attorney

## UNITED STATES PATENT OFFICE.

YULEE A. DYER, OF CAVE SPRING, GEORGIA.

## PROCESS AND APPARATUS FOR MELTING IRON.

Application filed February 4, 1925. Serial No. 6,784.

This invention relates to improvements in melting metals such, for instance, as iron.

An object of the invention, broadly, is twofold, in that it is desired to provide a melting apparatus and method with which, first, an appreciable saving in the quantity of fuel consumed is automatically effected, and second, in which the quality of the resulting metallic product will be materially improved. More specifically, the invention contemplates an apparatus wherein there is one cupola or furnace in which a portion of the metal is melted and a second adjoining cupola or furnace to which the waste products of combustion from the first cupola or furnace are conveyed and passed through a layer of fuel in the presence of additional metal to be melted.

In this way the quantity of fuel required in the second cupola or furnace in particular, is automatically reduced approximately fifty per cent, and the quantity of sulphur and other undesirable elements contained in the fuel, are likewise greatly precluded from contaminating the metal. This results in a higher grade product being obtained from both the first and second cupola or furnace, but especially more pronounced from the second cupola or furnace.

In the preferred method of practicing the present invention, alternate layers or charges of solid carbonaceous material to be combusted and metal to be melted are placed in the first cupola or furnace, into which either cold or preheated air is blown, the air entering the cupola or furnace under the lowermost layer or bed of carbonaceous material through which it is forced to produce combustion to melt the upper layers of metal within the cupola or furnace chamber. The hot escaping gases given off from the first cupola or furnace are then conveyed directly into a second cupola or furnace unit, through a conduit connecting the two units. Transference of these hot gases is aided by mechanically produced pressure, the gases first entering a gas belt surrounding the second cupola or furnace, and then enter interior of cupola or fur-

nace from said belt by way of a series of ports encircling the second cupola or furnace. These ports are located in the cupola or furnace wall at a point where the hot gases will enter below, and then pass through a comparatively thin bed of carbonaceous material which is combusted to melt relatively large layers of metal in the second cupola or furnace, the layers of carbonaceous material and metal in the second cupola or furnace being arranged alternately as in the first cupola or furnace.

This process, which may be termed a "twin-unit process", or "automatic recuperation process", may be practiced in various types of apparatus, the specific form shown in the present instance being illustrative only and highly diagrammatic.

The figure in the drawing is a general cross section, partly in side elevation, through the two melting units and their accessories.

As illustrated in the drawings, there is a melting cupola or melting furnace 10 closed at the top, the fuel and metal to be melted being fed into the combustion chamber of the cupola or furnace through a valve type charging box 12 of either automatic or hand type regulation. It will be understood that a bed charge or layer of fuel is first fed through the door 12, then a layer of metal to be melted, and then intermediate layers of fuel and metal, alternately. The second cupola or furnace, or melting unit, is indicated at 13, the wall of this unit being provided with suitably aligned charging doors 14, 15, through which layers of fuel and metal to be melted may be fed either automatically, or by hand, so as to place alternate layers of the fuel and metal in the combustion chamber of the cupola or furnace, the bottom layer or bed in this cupola or furnace also being of carbonaceous fuel.

Either cold or preheated air for aiding combustion in the first cupola or furnace is delivered by any desirable mechanism to and through a windpipe 16 communicating with a windbox 17 surrounding said cupola

or furnace, from which box the air flows into the interior of the cupola or furnace through a plurality of tuyères 18 arranged around the cupola or furnace wall in accordance with the usual practice. Surrounding the base of the second cupola or furnace 13 is a gas belt 19, which communicates with the interior of the cupola or furnace through a series of ports 20 in the cupola or furnace wall. The hot waste gases passing off from the cupola or furnace 10 are adapted to be removed and conveyed to this gas belt 19, from which they will flow into the second cupola or furnace 13 at a point beneath the lower layer of fuel in the latter, for burning or recuperation purposes. Preferably the passage 22, through which the gases flow from cupola or furnace 10 to gas belt 19, is so arranged with respect to cupola or furnace 10 that the wall of the latter will function as a baffle 21, over which the gases must pass before reaching the gas belt 19. However, if desired, a plurality of ports 21<sup>a</sup> may be provided in the wall 21 of the cupola or furnace so that said gases may flow more directly into the passage 22. To aid combustion in the second cupola or furnace 13 suitable air connections, indicated diagrammatically by the air inlet pipe 23, may be provided for supplying air to the passage 22.

The general operating plan or method practiced with this melting apparatus is as follows: The melting process in cupola or furnace 10 consists of charging alternate layers of carbonaceous material and metal, the lowermost layer or bed being one composed of carbonaceous material. This lower layer of fuel approximates a depth of about twenty-two inches above the tuyères 18. Upon combustion of the fuel in the cupola or furnace 10 the metal, which will become molten, and the usual slag, will pass out of a tap hole and flow down the tap spout 24 to the usual container, such as ladle 25, the slag being forced over the top of the side of the spout by the ordinary skim method. The waste gases, which would ordinarily pass off unused from cupola or furnace 10, are conveyed through the passage 22, either after passing over or through baffle wall 21, to the gas belt 19, the proper quantity of free or excess air oxygen (if necessary) to carry on combustion in the second cupola or furnace 13 having, in the meantime, been delivered to the said gases through the air supply connection 23. From the gas belt 19, the gases, with the combined air, pass through the ports 20 into the second cupola or furnace 13, where they not only aid in combusting the carbonaceous fuel in the second cupola or furnace, but also supply sensible heat units to assist in heating and melting upper metal charges in the

second cupola or furnace. The metal thus melted in the second cupola or furnace consistently flows from the cupola or furnace proper through an outlet 26 into the forehearth 27, and is finally tapped out at spout 28 into a container such as a bull ladle 29.

By utilizing the sensible heat units supplied by the waste hot gases coming into the second cupola or furnace, the layers of fuel used in that cupola or furnace, are, as a natural sequence to such operation, quite thin compared to those in the first cupola or furnace; the total quantity of fuel consumed in the melting process carried on in the second cupola or furnace, is thereby greatly reduced, this reduction amounting to approximately sixty per cent, by weight, in the case of the first lowermost layer or bed, and fifty per cent, by weight, in subsequent or intermediate charges of fuel. This natural reduction in the quantity of fuel consumed, is quite an advantage in that the cost of operation is greatly curtailed, but this is by no means the only advantage resulting from the present process. A second resulting advantage, and a worthy one, lies in the improved quality of the melted metal obtained from the second cupola or furnace. The metal obtained from the second cupola or furnace has been found, in actual practice, to be more dense and homogeneous, making a product that can be easily machined and which possesses an increased strength approximating fifty per cent to sixty per cent over metal melted in an ordinary single-unit cupola or furnace. This highly desirable result is obtained by reason of the fact that such a small quantity of sulphur and other contaminating elements is present in the second cupola or furnace. That is, the quantity of fuel necessary to be used in the second cupola or furnace having been reduced approximately one-half, the quantity of sulphur and other contaminating elements, which are a residue of burned fuel, are not absorbed by the metal being melted in that cupola or furnace. If, and when, desired, the metal from the two cupolas or furnaces may be conveyed to a single container, thereby making a mixture of any desired analysis within the scope of rational cupola practice.

What I claim is:

1. The process of melting metal, which consists in charging one combustion chamber with a comparatively deep bed of carbonaceous material, combusting said material in the presence of a supply of air and a body of metal to be melted, and then transferring or conveying the hot waste gases from said chamber directly to a second combustion chamber and there passing said hot waste gases under and through a comparatively thin layer of carbonaceous material in the presence of additional metal to be

melted, whereby the quantity of fuel required in said second chamber is materially reduced.

2. The process of melting metal, which consists in charging one combustion chamber with a comparatively deep bed of carbonaceous material, combusting said material in the presence of a supply of air and a body of metal to be melted, conveying the hot waste gases directly to a second combustion chamber, introducing a supply of additional air to said gases at a point intermediate the two chambers, and then passing said gases and additional air under and through a comparatively thin layer of carbonaceous material in the presence of additional metal to be melted, whereby the quantity of carbonaceous material required in the second chamber and the quantity of sulphur and other contaminating elements coming in contact with the metal in said second chamber, are materially reduced.

3. The process of melting metal, which consists in charging one combustion chamber with a comparatively deep bed of carbonaceous material, above which layers of metal to be melted and carbonaceous fuel to be combusted, are arranged alternately, combusting said carbonaceous material in the presence of a supply of air and the body of metal to be melted, and then transferring, or conveying, the hot waste gases from said chamber directly to a second combustion chamber, and there passing said hot waste gases under and through a comparatively thin layer of carbonaceous material, above which several alternate layers of metal to be melted and thin layers of carbonaceous fuel to be combusted, are arranged alternately, whereby the quantity of fuel required in said second chamber is materially reduced, and the quality of the melted metal is materially improved.

4. The process of melting metal, which consists in charging one combustion chamber with a comparatively deep bed of carbonaceous material, above which are alternately placed layers of metal to be melted and layers of carbonaceous fuel to be combusted, respectively, combusting said carbonaceous material in the presence of a supply of air and a body of metal to be melted, conveying the hot waste gases, after the same have served their purpose in said combustion chamber, from said combustion chamber directly into a second combustion chamber, introducing a supply of additional air to said gases at a point intermediate the said two chambers, and then passing said gases and additional air under and through a comparatively thin bed of carbonaceous material, above which are arranged, or placed, alternate layers of metal to be melted and thin layers of carbonaceous material to be combusted, whereby the quantity of carbona-

ceous material required in the second chamber and the quantity of sulphur and other contaminating elements, contained in said carbonaceous material, coming in contact with the metal in said second chamber, are 70 materially reduced, and the quality of the metal melted in said second chamber is materially improved.

5. The process of melting metal, which consists in charging one combustion chamber with a comparatively deep bed of carbonaceous fuel, above which are placed alternate layers of metal to be melted and carbonaceous fuel, so that a layer of said metal to be melted will always remain above 75 a layer of said carbonaceous fuel to be combusted, combusting said carbonaceous fuel in the presence of a layer of said metal to be melted and a supply of air forced into said combustion chamber under mechanical 80 pressure, conveying the hot waste gases from said combustion chamber directly to a second combustion chamber, introducing a supply of additional air to said gases at a point intermediate the two said chambers, and 85 then passing said gases and additional air into a second combustion chamber containing a thin lower layer, or bed, of carbonaceous fuel, directly above which are arranged, first, a layer of metal to be melted, 90 and then alternate thin layers of carbonaceous fuel and metal to be melted, so that a thin layer of said carbonaceous fuel will always remain immediately under and 95 against one of said layers of metal, which 100 said waste gases and additional air so passed into said combustion chamber are forced under and through said alternate layers of carbonaceous fuel to be combusted and metal to be melted, in said second combustion chamber, whereby the quantity of carbonaceous fuel required in the said second combustion chamber and the quantity of sulphur and other contaminating elements coming in contact with said metal to be melted in said 110 second combustion chamber are materially reduced.

6. The process of melting metal, which consists in charging a cupola furnace with a comparatively deep bed of carbonaceous material, combusting said material in the presence of a supply of air and a body of metal to be melted, and then transferring or conveying the hot waste gases from said cupola to the combustion chamber of a second cupola and there passing said hot waste gases under and through a comparatively thin layer of carbonaceous material in the presence of additional metal to be melted, whereby the quantity of fuel required in said second chamber is materially reduced.

7. The process of melting metal, which consists in charging a cupola furnace with a comparatively deep bed of carbonaceous material, combusting said material in the

presence of a supply of air and a body of metal to be melted, conveying the hot waste gases to the second cupola furnace, introducing a supply of additional air to said hot waste gases during their travel from the first cupola to the second cupola, and then passing said hot waste gases and additional air through a comparatively thin lay-

er of carbonaceous material in the presence of additional metal to be melted, whereby the quantity of carbonaceous material required in the second chamber and the quantity of sulphur and other contaminating elements coming in contact with the metal in the second cupola are materially reduced.

YULEE A. DYER.